

## UNITED STATES PATENT OFFICE.

JAQUES EDWIN BRANDENBERGER, OF PARIS, FRANCE, ASSIGNOR TO SOCIETE INDUSTRIELLE POUR L'APPLICATION DE BREVETS ET PROCEDES, OF RUEIL, FRANCE.

## PRODUCTION OF HYDRATED CELLULOSES.

No Drawing.

Application filed June 4, 1923. Serial No. 643,438.

*To all whom it may concern:*

Be it known that I, JAQUES EDWIN BRANDENBERGER, citizen of Helvetia, residing at Paris, Seine, France, have invented certain new and useful Improvements in or Relating to the Production of Hydrated Celluloses, of which the following is a specification.

The present invention relates to improvements in or connected with the production of hydrated celluloses.

Celluloses generally called cellulose hydrates amongst which may be mentioned for example mercerized cotton, sulphurized paper, the celluloses obtained from the regeneration of their cellulosic solutions, and the like, exhibit during use certain serious drawbacks which are due to the amount of water which they absorb.

Thus, for example, in the case of mercerized cotton, it will be found that it has a greater affinity for colouring matters than non-hydrated celluloses. When a mixed fabric consisting of ordinary cotton and mercerized cotton, is to be dyed, this property renders it impossible to obtain a uniform colouring, the mercerized cotton absorbing more colour than the ordinary cotton.

This drawback is considerably aggravated with artificial fabrics, if the latter are used together with ordinary cotton. Moreover, in consequence of the greater absorptive power for liquids of hydrated celluloses, these latter are more easily deformed than the non-hydrated celluloses. As a matter of fact, they stretch more when they are humidified, and on drying, in consequence of their shrinkage being greater than that of ordinary cellulose, the treated fabrics are often deformed and have not that finished appearance of non-hydrated celluloses.

If now—also by way of example—a cellulose is considered which has been regenerated from a cellulosic solution in the form of a film and has been brought to its state of equilibrium by moistening followed by drying, in its free state, and if for any application it is found necessary to moisten said film, it absorbs an amount of water representing for example 80% of its weight in a dry state, and its dimensions will be

found to increase as regards length, at least 6%, and in the other direction, i. e., as regards width, at least 12%. In consequence of the final drying in its free state, the film is deformed, and cannot be used for certain important purposes, for which it could be used if these disadvantages were not present.

It is conceivable—and has as a matter of fact often been sought for since hydrated cellulose came into use—how important it would be to diminish the absorptive power of the hydrated cellulose for water as well as for colouring matters and other chemical products or generally for any aqueous solutions.

The object of the present invention is a treatment to which hydrated cellulose of any kind is subjected after its manufacture and drying, which treatment consists in subjecting the product in its dry state to the action of dry saturated steam in a closed vessel. The term "product in its dry state" is intended to mean the product containing its natural hygroscopic water. The effect obtained is the more rapid as the temperature, and consequently the pressure of the steam are increased. If, for example steam of 2 kg. pressure is allowed to act on a mass of cellulose hydrate films rolled up on a spindle in a layer of 30 mm. thickness, the action is complete after two hours. It would be finished within a shorter period in the case of a single layer of film.

The operation can be carried out with a film as soon as it is manufactured, or after it has already been subjected to one or more moistening and drying operations in its free state or under tension.

The product obtained when considered as being in its state of equilibrium, i. e., moist, and thereupon dried in its free state, when re-moistened exhibits increases of dimensions which are substantially only half of those which it would have shown without the steam treatment, that is to say, for example 3% and 6%, instead of 6% and 12% in the case of the cellulose film above-mentioned. Moreover, the rapidity with which the water is taken up by the film is considerably diminished, being reduced from 80% to 40% in the aforesaid case.

The action is much slower with saturated

steam at 100° C. or below. There is no advantage in using very high pressures, because a final invariable state is always obtained, provided the action is of sufficient duration. The thus treated films are deformed much less when they are dried in a free state.

An analogous effect is observed on artificial cellulosic textile fabrics. Their increase in length on moistening is diminished in the same proportion. Moreover, the affinity of the thus treated product for direct colours is reduced. It is actually known that artificial textile fabrics absorb in the same bath up to three times the amount of colouring matters absorbed by cotton.

This diminution in the affinity of the artificial textile fabrics for colouring matters is of great advantage in case it is desired to dye with equal effect a mixed fabric of cotton and artificial fibres. This is also a means for equalizing the shades of the colouring since it is known that slight differences in the treatment during the manufacture of artificial textile material may produce very decided differences in the dyeing for which there has heretofore been no efficient remedy.

The treatment of the dry cellulosic product with dry saturated steam, seems actually to have the effect of bringing together the different states of the cellulose to a state having constant properties corresponding to the ordinary cellulose of natural cotton. The action is produced on any cellulose even if it has been partially hydrated by the action of acids, bases and salts. Thus for example the action takes place on bleached or mercerized cotton. The dry saturated steam has no action on hydrated celluloses which have been previously moistened, this being due to the fact that such celluloses contain more than their normal content of moisture. The strength of the product when moist is also increased by the above treatment.

The effect produced by the present invention has nothing in common with the ordinary known treatment of artificial textile fibres by chemical reaction which is generally intended only to increase the strength of the product when moist.

If for example, the operation is effected on a compact mass of cellulose on rollers, it is evident that a simple heating in a closed vessel exhausted of air will also effect the result specified, owing to the rapid saturation of the vessel by part of the hygroscopic water, which is always retained in cellulose.

It should finally be remarked that the use of dry saturated steam upon celluloses having a normal moisture content is indispensable, because superheated steam acting upon the hydrated celluloses gives a result which apparently does not differ substantially from that obtained by hot air, that is to say a simple drying effect which removes the hygro-

scopic water and yields a breakable and non-elastic product. In order to carry out the process two conditions are therefore essential. First, it is necessary to use saturated steam and not superheated steam upon celluloses of normal moisture content, and secondly it is necessary that this saturated steam should be dry, without which it would moisten the cellulose and no action would be obtained. Moreover, as already stated, it is necessary that the product treated with the steam should be absolutely dry.

It should be understood that the term "cellulose hydrates" includes cellulose hydrates of any kind, such as mercerized cotton, sulphurized paper and cellulose obtained by regeneration from cellulosic solutions and the like, irrespective of the form in which the hydrated cellulose is produced during the manufacture.

Having now particularly described and ascertained the nature of my said invention as well as the manner in which the same is to be performed, what I claim as new is:

1. Process for dehydrating cellulose hydrates, which comprises subjecting said celluloses hydrates in an air-dried condition to the action of dry saturated steam. 90

2. Process for dehydrating cellulose hydrates, which comprises subjecting said cellulose hydrates in an air-dried condition to the action of dry saturated steam in a closed vessel. 95

3. Process for dehydrating cellulose hydrates, which comprises subjecting said cellulose hydrates in an air-dried condition to the action of dry saturated steam under pressure. 100

4. Process for dehydrating cellulose hydrates in a manufactured state, which comprises subjecting said cellulose hydrates in an air-dried condition to the action of dry saturated steam. 105

5. Process for dehydrating cellulose hydrates in a manufactured state, which comprises subjecting said cellulose hydrates in an air-dried condition to the action of dry saturated steam in a closed vessel. 110

6. Process for dehydrating cellulose hydrates in a manufactured state, which comprises subjecting said cellulose hydrates in an air-dried condition to the action of dry saturated steam under pressure. 115

7. Process for dehydrating cellulose hydrates immediately after being manufactured, which comprises subjecting said cellulose hydrates in an air-dried condition to the action of dry saturated steam. 120

8. Process for dehydrating cellulose hydrates immediately after being manufactured, which comprises subjecting said cellulose hydrates in an air-dried condition to the action of dry saturated steam in a closed vessel. 125

9. Process for dehydrating cellulose hy- 130

drates immediately after being manufactured, which comprises subjecting said cellulose hydrates in an air-dried condition to the action of dry saturated steam under 5 pressure.

10. Process for dehydrating cellulose hydrates, which comprises subjecting said cellulose hydrates to moistening and drying operations and thereupon whilst in an air-dried condition, to the action of dry saturated steam.

11. Process for dehydrating cellulose hydrates, which comprises subjecting said cellulose hydrates to moistening and drying 15 operations and thereupon whilst in an air-dried condition, to the action of dry saturated steam in a closed vessel.

12. Process for dehydrating cellulose hydrates, which comprises subjecting said 20 cellulose hydrates to moistening and drying operations and thereupon whilst in an air-dried condition, to the action of dry saturated steam under pressure.

13. Process for dehydrating cellulose hydrates in a manufactured state, which comprises subjecting said cellulose hydrates to moistening and drying operations and thereupon whilst in an air-dried condition, 25 to the action of dry saturated steam.

30 14. Process for dehydrating cellulose hydrates in a manufactured state, which comprises subjecting said cellulose hydrates to moistening and drying operations and thereupon whilst in an air-dried condition, 35 to the action of dry saturated steam in a closed vessel.

15. Process for dehydrating cellulose hydrates in a manufactured state, which comprises subjecting said cellulose hydrates to moistening and drying operations and thereupon whilst in an air-dried condition, to the action of dry saturated steam under 40 pressure.

45 16. Process for dehydrating cellulose hydrates which comprises subjecting said cellulose hydrates in an air-dried condition and in a tensioned state to the action of dry saturated steam.

50 17. Process for dehydrating cellulose hydrates which comprises subjecting said cellulose hydrates in an air-dried condition

and in a tensioned state to the action of dry saturated steam in a closed vessel.

18. Process for dehydrating cellulose hydrates which comprises subjecting said 55 cellulose hydrates in an air-dried condition and in a tensioned state to the action of dry saturated steam under pressure.

19. Process for dehydrating cellulose hydrates in a manufactured state, which comprises subjecting said cellulose hydrates to moistening and drying operations and thereupon whilst in an air-dried condition and in a tensioned state, to the action of 60 dry saturated steam.

65 20. Process for dehydrating cellulose hydrates in a manufactured state, which comprises subjecting said cellulose hydrates to moistening and drying operations and thereupon whilst in an air-dried condition 70 and in a tensioned state, to the action of dry saturated steam in a closed vessel.

75 21. Process for dehydrating cellulose hydrates in a manufactured state, which comprises subjecting said cellulose hydrates to moistening and drying operations and thereupon whilst in an air-dried condition and in a tensioned state, to the action of dry saturated steam under pressure.

80 22. A cellulose hydrate having a reduced absorptive capacity for liquid on moistening and a decreased liability to deformation during such moistening and drying operations to which it may be subjected, but otherwise retaining all its original physical properties, said cellulose hydrate being produced by subjecting cellulose hydrates in an air-dried condition to the action of dry saturated steam.

85 90 23. A cellulose hydrate in a manufactured state having a reduced absorptive capacity for liquid on moistening and a decreased liability to deformation during such moistening and drying operations to which it may be subjected, but otherwise retaining all its 95 original physical properties, said cellulose hydrate being produced by subjecting cellulose hydrates in an air-dried condition to the action of dry saturated steam in a closed vessel under pressure.

100 In testimony whereof I affix my signature.

JAQUES EDWIN BRANDENBERGER.